

Dec. 12, 1950

D. A. HOWES ET AL

2,534,025

PRODUCTION OF AVIATION OR MOTOR FUELS

Filed Dec. 15, 1948



Inventor

Donald Albert Howes  
Thomas Tait

By Morgan, Trumgar & Durham  
Attorneys

## UNITED STATES PATENT OFFICE

2,534,025

## PRODUCTION OF AVIATION OR MOTOR FUELS

Donald A. Howes and Thomas Tait, Sunbury-on-Thames, England, assignors to Anglo-Iranian Oil Company Limited, London, England, a British joint-stock corporation

Application December 15, 1948, Serial No. 65,468  
In Great Britain May 5, 1941

10 Claims. (Cl. 196—78)

1

The invention relates to the production of high grade aviation or motor fuels or motor fuel constituents. More particularly the invention relates to the production of high grade motor fuel from feedstocks containing appreciable proportions of mono-olefines and di-olefines such as the cracked distillates produced in known thermal cracking or thermal reforming operations.

Such cracked distillates are unsuitable for use in aero-engines because of their liability to oxidation and deterioration in storage. It is among the objects of the invention so to treat such distillates that appreciable quantities of stable high grade aviation spirit may be obtained from them.

The invention is not limited to any particular method of producing the feedstock. The cracked distillate subjected to the process of the invention may for example be obtained from a crude stock and may comprise any fraction derived from a crude mineral oil ranging from naphtha to heavy residuum. Particularly good results are obtained however in the use as feedstocks of cracked distillates obtained in thermal reforming operations, in which the feedstocks are those generally known as naphthas having a boiling range approximating 70° C.—300° C. The thermal reforming conditions usually employed in such cases vary as to temperature between 480° C. and 700° C. and as to pressure between 100 and 2,000 lbs. per square inch. The condensable gases formed in the process, being C<sub>3</sub> and C<sub>4</sub> hydrocarbons may be recycled to the cracking still and mixed with the naphtha feed. In general the cracked distillate so produced will have an octane number (C. F. R. Motor Method) of from 65 to as high as 90 or even higher, according to the character or composition of the naphtha processed and the reforming conditions employed. In the nature of the case products of higher octane number require the use of more drastic conditions of reforming in the use of higher temperatures in the ranges.

According to the invention a feedstock containing mono-olefines and/or di-olefines, such as the cracked distillates referred to, is submitted to hydrogenation to convert the mono-olefines and/or di-olefines into the corresponding paraffin or naphthene hydrocarbons, and the treated material including the saturated products are thereupon fractionated for the separation of hydrocarbons or fractions of low octane member consisting mainly of the normal paraffins and simple branched chain paraffins of low octane number, and for the recovery of hydrocarbons or fractions of high octane number consisting mainly of

2

naphthene hydrocarbons and branched chain paraffin hydrocarbons of high octane number, under the conditions hereinafter more particularly described; and the hydrocarbons or fractions of high octane number recovered may be blended together, and with hydrocarbons such as toluene, xylene and higher aromatic hydrocarbons recovered in known manner as by solvent extraction from the recovered hydrogenated product or a fraction thereof. The high octane number hydrocarbons or fractions may be used individually or together in varying proportions as constituents of a high grade motor or aviation fuel.

15 The feedstock may be first desulphurized or may be desulphurized under the conditions of hydrogenation. The preliminary desulphurization is however only necessary if the feedstock contains a proportion of sulphur compounds injurious to the hydrogenation catalyst employed.

20 The invention comprises the process conditions hereinafter described.

In carrying the invention into effect the hydrogenation treatment may be carried out on a cracked distillate having for example a final boiling point of 200° C. to 300° C. at a temperature within the range 150° C. to 300° C. and at a space velocity of 0.5 to 5.0 volumes per volume of catalyst per hour. Hydrogen is advantageously employed in excess, and the hydrogenating catalyst may conveniently consist of or contain a mixture of tungsten and nickel sulphides, or cobalt molybdate or nickel molybdate or reduced iron oxide or a mixture of alumina and nickel oxide.

35 The hydrogenated product may ordinarily contain a small quantity of hydrogen sulphide in solution, which may be removed by washing the hydrogenated product with an alkaline solution such as a solution of caustic soda. The mono-olefines and/or di-olefines of the feedstock are converted under the conditions of treatment into the corresponding paraffin and naphthene hydrocarbons by simple addition of hydrogen, unaccompanied by any substantial formation of hydrocarbons of lower molecular weight.

45 Where the feedstock has a sulphur content injurious to the catalyst that may be employed for its hydrogenation, the feedstock may be first subjected to treatment for the substantial removal of the sulphur compounds. Hydrogenation catalysts are affected in a varying degree by the presence of sulphur compounds. Thus simple reduced nickel catalysts are rapidly poisoned by very small amounts of sulphur compounds, for example 0.01% or less, while mixtures of tungsten and

nickel sulphides and other hydrogenation catalysts are resistant to sulphur and are not affected appreciably by contents of sulphur up to 0.1% or more. The sulphur compounds are thus converted to hydrogen sulphide whereby desulphurization may proceed simultaneously with hydrogenation.

Desulphurization treatment when required by the character of the feedstock may be carried out by passing the cracked distillate feedstock after vaporization over a desulphurizing catalyst such for example as granular bauxite or Super Filtral at a temperature within the range 530° C. to 700° C., and at a throughput of from 0.5 to 10 liquid volumes per volume of catalyst per hour, 15 in the absence of hydrogen. Alternatively desulphurizing catalysts comprising mixtures of molybdc oxide and alumina, or chromic oxide and alumina may be employed under the same reaction conditions, but in the presence of added hydrogen. In this manner the sulphur content of the cracked distillate may be reduced from for example 0.1% to less than 0.001%.

The hydrogenated product may then be fractionated under conditions of precision in fractionation determined to insure control of top and bottom temperatures, reflux ratios and pressures in the fractionating columns and in the use of the equivalent of 50 or more theoretical plates, whereby the normal paraffin hydrocarbons or fractions rich in such constituents are removed. Such normal hydrocarbons present in the feedstock or formed during the treatment that results in the simple saturation of straight chain olefine hydrocarbons, are of low octane number, 35 as indicated by the following figures:

|                | Octane number<br>(C. F. R. Motor) |
|----------------|-----------------------------------|
| Normal pentane | 61                                |
| Normal hexane  | 25                                |
| Normal heptane | 0                                 |
| Normal octane  | 17                                |
| Normal nonane  | 45                                |

Their removal thus results in a marked increase in the octane number of such hydrocarbons or fractions recovered.

The hydrogenated product may be fractionated to form a lighter and a heavier fraction and that part of the hydrogenated product boiling above about 100° C. may be treated with a selective solvent for the recovery of aromatic hydrocarbons such as toluene, xylene, ethyl benzene and higher aromatic hydrocarbons. For this purpose liquid sulphur dioxide may advantageously be used and the treatment carried out in known manner at a low temperature of from -10° C. to -80° C., whereby the aromatic hydrocarbons are recovered in a high concentration. The lighter fraction may be fractionated under the conditions hereinbefore described for the separation of normal paraffins and simple branched chain paraffins of low octane number and for the recovery under the conditions described of branched chain paraffin and naphthene hydrocarbons of high octane number for blending in the production of fuels.

Aviation fuels of high octane number may be prepared by blending the aromatic hydrocarbons thus recovered together with other fractions of the hydrogenated product such as branched chain paraffin hydrocarbons and naphthenes that may have been recovered from that part of the hydrogenated product boiling up to 100° C. and from which the normal paraffins or fractions rich

in normal paraffins have been removed in the manner under the conditions described.

The invention is diagrammatically illustrated by way of example in the accompanying drawing.

In carrying the invention into effect as illustrated in the accompanying drawing a feedstock, such, for example, as a distillate produced in the thermal cracking or thermal reforming operation is desulphurized under known conditions such as hereinbefore described in a preliminary treatment stage *k* if it contains an appreciable proportion of sulphur, and is thereupon hydrogenated in a known manner in a succeeding stage *l* under conditions such as hereinbefore described for the conversion of the mono-olefine and di-olefine content into corresponding paraffin and naphthene hydrocarbons.

The hydrogenated product is then fractionated in a fractionator *L* to obtain a light fraction as an overhead product and a heavier fraction as a bottoms product.

The bottoms product of the fractionator *L*, which may advantageously be that part of the hydrogenated product boiling above 100° C., is passed for solvent extraction of its aromatic hydrocarbon content through the solvent extraction and separating plant *m*, which operates in known manner, the material flowing successively first into a mixing tank in which it is contacted with liquid sulphur dioxide under known conditions, whereupon the mixture passes into a settling tank for the settlement and separation of the extract and raffinate phases. The aromatic extract thence passes as feed to a column for the removal of the liquid sulphur dioxide as overhead and the aromatic extract as bottoms, which latter may pass to storage for eventual use of the material as a fuel blending constituent in the proportions that may be stipulated by fuel specifications, while the raffinate passes as feed to a column where the sulphur dioxide is separated and the raffinate passes to storage.

The overhead product of the fractionator *L* is passed to the first of a series of fractionating columns *a*, *b*, *c*, *d* and *e* for the separation under conditions of precision in fractionation of hydrocarbons or fractions consisting mainly of the normal paraffins and simple branched chain paraffins of low octane number, and for the recovery of hydrocarbons or fractions of high octane number consisting mainly of naphthene hydrocarbons and branched chain paraffin hydrocarbons of high octane number.

Each of the columns is provided for example with the equivalent of a moderately large number of theoretical plates not substantially less than 50 theoretical plates and a moderate reflux ratio maintained in operation of the columns for example of 15:1, and top and bottom temperatures maintained in the columns under control by analysis and the use of laboratory equipment and a moderate pressure applied in the column in which isopentane is recovered, whereby the operating conditions may be precisely controlled in the respective columns having regard to the determinations thus made as to composition.

The temperature conditions are determined in the columns such that an isopentane fraction is recovered in the column *a* as overhead from normal pentane and higher hydrocarbons which leave as bottoms. The latter thence passes into the column *b* at a mid-position in its length where the operating conditions are so determined that normal pentane is separated as overhead and higher hydrocarbons leave as bottoms. The lat-

ter then passes to a mid-position in the column *c* in which an "iso-hexane" fraction is recovered as overhead having an approximate boiling range of 45-64° C. including cyclopentane and the four hexane isomers to the substantial exclusion of normal hexane which leaves the column *c* with the higher hydrocarbons as bottoms, to enter the next column *d* at a mid-position, where the normal hexane fraction is separated as overhead and the remainder as bottoms. The latter then passes in a mid-position to the column *e*, where at a moderate reflux ratio of approximately 10:1 a recovery of an "isoheptane" fraction is made as overhead, having the approximate boiling range of 72-92° C. comprising the content of cyclic hydrocarbons and branched chain hydrocarbons boiling in that range to the exclusion of any substantial proportion of 2-methyl hexane, 3-methyl hexane, 3-ethyl pentane and normal heptane which leaves the column *e* through the pipe *e*<sup>1</sup> together with the hydrocarbons boiling beyond that range.

The high grade overhead fractions from the columns *a*, *c* and *e* pass by the respective lines *a*<sup>1</sup>, *c*<sup>1</sup> and *e*<sup>1</sup> to the respective storage vessels *a*<sup>2</sup>, *c*<sup>2</sup>, and *e*<sup>2</sup> whence they may be withdrawn as blending constituents for use with the aromatic extract hereinbefore described in the proportions that may be stipulated by fuel specifications.

The normal pentane and normal hexane fractions leaving as overhead respectively from the columns *b* and *d* may pass by the pipe line *b*<sup>1</sup> to storage.

It will be understood that the extent of fractionation will depend upon the initial boiling point of the feedstock. Thus according to its composition, the feedstock may only require fractionation in the columns *b*, *c*, *d* and *e* or other smaller number of columns according to its content of normal paraffin hydrocarbons and of its content of isopentane and of the "isohexane" and "iso-heptane" fractions.

This application is a continuation-in-part of our copending application, Serial Number 444,260, filed May 23, 1942, and now abandoned, for "Improvements relating to the production of aviation or motor fuels."

What is claimed is:

1. A process for the production of blending constituents of an aviation or motor fuel of high octane number from a substantially sulphur-free cracked petroleum distillate containing mono-olefines and di-olefines, comprising subjecting the sulphur-free feedstock to hydrogenation for the conversion of the mono-olefine and di-olefine content into corresponding paraffin and naphthene hydrocarbons by simple addition of hydrogen, separating the hydrogenated cracked distillate into a lighter fraction boiling up to about 100° C. and into a heavier fraction, subjecting said lighter fraction of the hydrogenated cracked distillate to fractionation for the separation therefrom of at least one normal fraction, namely normal heptane together with the content of said lighter fraction boiling beyond about 92° C. and for the recovery from said lighter fraction of at least one fraction of high octane number, namely a fraction having an approximate boiling range of about 72° C. to about 92° C. comprising the content of cyclic hydrocarbons and branched chain hydrocarbons boiling in that range to the exclusion of any substantial proportion of 2-methyl hexane, 3-methyl hexane, 3-ethyl pentane and normal heptane, the fractionations being carried out under conditions of precision in the main-

tenance of determined top and bottom temperatures and pressure, in the use of columns having the equivalent of a moderately large number of theoretical plates not substantially less than 50 theoretical plates, and a high reflux ratio, in general not substantially less than 15:1, and subjecting the said heavier fraction of the hydrogenated cracked distillate boiling beyond about 100° C. to solvent extraction for the recovery from said heavier fraction of an aromatic hydrocarbon extract as an additional blending constituent.

2. A process as specified in claim 1, in which the material fed to the columns is analyzed and the operating conditions precisely controlled in the columns having regard to the determinations made.

3. A process for the production of blending constituents of an aviation or motor fuel of high octane number from a cracked petroleum distillate as specified in claim 1, in which the said lighter fraction of the hydrogenated cracked distillate before being fractionated for the separation of normal heptane, is fractionated under the same conditions of precision in fractionation for the recovery of a fraction of high octane number having approximately a boiling range of 45°-64° C. comprising substantially the content in the hydrogenated cracked distillate, of cyclopentane together with the dimethyl butanes and the methyl pentanes boiling in that range as an additional blending constituent.

4. A process for the production of blending constituents of an aviation or motor fuel of high octane number from a cracked petroleum distillate as specified in claim 1, in which said lighter fraction of the hydrogenated cracked distillate before being fractionated for the separation of normal heptane, is fractionated under the same conditions of precision in fractionation for the recovery of a fraction of high octane number having approximately a boiling range of 45°-64° C. comprising substantially the content in the hydrogenated cracked distillate, or cyclopentane together with the dimethyl butanes and the methyl pentanes boiling in that range as an additional blending constituent and in which the material fed to the columns is analyzed, and the operating conditions precisely controlled in the columns having regard to the determinations made.

5. A process for the production of blending constituents of an aviation or motor fuel of high octane number from a cracked petroleum distillate as specified in claim 1, in which the said lighter fraction of the hydrogenated cracked distillate before being fractionated for the separation of normal heptane is fractionated under the same conditions of precision in fractionation for the separation of normal pentane, for the recovery of an additional fraction of high octane number having approximately a boiling range of 45°-64° C., comprising substantially the content in the distillate of cyclopentane together with the di-methyl butanes and the methyl pentanes boiling in that range, as a blending constituent, and for the recovery of the content of isopentane, as a blending constituent.

6. A process for the production of blending constituents of an aviation or motor fuel of high octane number from a cracked petroleum distillate as specified in claim 1, in which said lighter fraction of the hydrogenated cracked distillate before being fractionated for the separation of normal heptane is fractionated under the same conditions of precision in fractionation, for the separation of normal pentane and

normal hexane, for the recovery of a fraction of high octane number having approximately a boiling range of 45°-64° C., comprising substantially the content in the distillate of cyclopentane together with the di-methyl butanes and the methyl pentanes boiling in that range, as a blending constituent, and for the recovery of the content of isopentane as a blending constituent, and in which the material fed to the column is analyzed, and the operating conditions precisely controlled in the columns having regard to the determinations made.

7. A process for the production of blending constituents of an aviation or motor fuel of high octane number from a cracked and hydrogenated distillate as specified in claim 1, in which the fraction having a boiling range of 72° to about 92° C. is recovered in a column operating at a reflux ratio of substantially 10:1.

8. A process for the production of blending constituents of an aviation or motor fuel as specified in claim 1, in which the cracked distillate has a final boiling point of from 200° C. to 300° C. and is hydrogenated at a temperature in the range 150° C.-300° C. and at a space velocity of 0.5 to 5.0 vols. per vol. of catalyst per hour.

9. A process for the production of blending constituents of an aviation or motor fuel as specified in claim 1, in which the cracked feedstock is hydrogenated in the presence of hydrogen in excess.

10. A process for the production of blending constituents of an aviation or motor fuel of high octane number from a substantially sulfur-free cracked petroleum distillate containing mono-olefines and diolefines comprising the steps of hydrogenating the feedstock for the conversion of the mono-olefine and diolefinic content into corresponding paraffin and naphthene

hydrocarbons by simple addition of hydrogen, subjecting the lighter portion of the hydrogenated product boiling up to about 100° C. to fractionation for the separation therefrom of at least one normal fraction, namely normal heptane together with the content of said lighter portion boiling beyond about 92° C. and for the recovery from said lighter portion of at least one fraction of high octane number, namely a fraction having an approximate boiling range of about 72° C. to about 92° C. comprising the content of cyclic hydrocarbons and branched chain hydrocarbons boiling in that range to the exclusion of any substantial proportion of 2-methyl hexane, 3-methyl hexane, 3-ethyl pentane and normal heptane, the fractionation being carried out under conditions of precision in the maintenance of determined top and bottom temperatures and pressure, in the use of columns having the equivalent of a moderately large number of theoretical plates not substantially less than 50 theoretical plates, and a high reflux ratio, in general not substantially less than 15:1.

DONALD A. HOWES.  
THOMAS TAITT.

#### REFERENCES CITED

The following references are of record in the file of this patent:

#### UNITED STATES PATENTS

| Number    | Name          | Date           |
|-----------|---------------|----------------|
| 2,055,455 | Taylor et al. | Sept. 22, 1936 |

#### OTHER REFERENCES

Petroleum Processing, vol. 2, No. 2 (Feb., 1947), pages 136, 139, 140, 142, 143, 145 and 146 (article by Birch, Docksey, and Dove on "Superfractionation").